

# United States Patent

[19]

Laskin et al.

[11] 3,967,042

[45] June 29, 1976

[54] **FUSER BLANKET**

[75] Inventors: **Harold B. Laskin**, New Brighton;  
**Robert H. Valentine**, St. Paul, both  
of Minn.

[73] Assignee: **Minnesota Mining and  
Manufacturing Company**, St. Paul,  
Minn.

[22] Filed: **Jan. 12, 1973**

[21] Appl. No.: **322,915**

[52] U.S. Cl..... **428/422; 428/447;**

**428/450; 432/61; 219/216; 427/261**

[51] Int. Cl.<sup>2</sup> ..... **B32B 27/00**

[58] Field of Search ..... **161/189, 206; 428/422,  
428/447, 450**

## [56] References Cited

### UNITED STATES PATENTS

|           |        |                |           |
|-----------|--------|----------------|-----------|
| 2,833,656 | 5/1958 | Sandt .....    | 161/189 X |
| 2,898,631 | 8/1959 | Jeffery .....  | 18/47.5   |
| 2,932,599 | 4/1960 | Dahlgren ..... | 161/189 X |

|           |         |                   |              |
|-----------|---------|-------------------|--------------|
| 3,051,677 | 8/1962  | Rexford .....     | 204/159.17 X |
| 3,146,799 | 9/1964  | Fekete .....      | 161/206 X    |
| 3,291,466 | 12/1966 | Aser et al. ....  | 432/61 X     |
| 3,296,063 | 1/1967  | Chandler .....    | 161/206 X    |
| 3,554,836 | 1/1971  | Steindorf .....   | 161/413 X    |
| 3,655,727 | 4/1972  | Patel et al. .... | 260/80.76 X  |

Primary Examiner—Marion E. McCamish

Assistant Examiner—Patricia C. Ives

Attorney, Agent, or Firm—Alexander, Sell, Steldt &  
DeLahunt

[57]

## ABSTRACT

A composite laminate structure is provided which is suitable for use as a fuser blanket in copiers or reproducers which are based on heat fixing of images on receptor surfaces. The structure is comprised of a dimensionally stable, heat conductive substrate having bonded to one surface thereof a thin, resiliently compressible layer of a fluorinated elastomeric polymer and an outer layer bonded thereto of a thin, resiliently compressible silicone elastomer.

7 Claims, 2 Drawing Figures





*FIG. 1*



*FIG. 2*

## FUSER BLANKET

## BACKGROUND OF THE INVENTION

This invention relates to the field of duplication wherein heat fixing systems for fixing images on powdered thermoplastic marking media to receptor surfaces, e.g. in high speed automatic copiers or reproducers, are utilized. More particularly it relates to an improved fusing blanket construction for use in such fixing systems.

The use of thermoplastic resin material in particulate form for the purpose of forming images on paper in copying machines or the like has generated various devices for adhering the particulate material to the desired receptor surfaces, especially in the form of sheets. It is necessary that the particulate resin material, hereinafter referred to as ink or toner powder, be fused or softened to a tacky state such that it can adhere to the receptor surface, and upon cooling will be bonded to the receptor surface to form images thereon. It is important in fixing the ink to the receptor surface that the ink is not disturbed as far as location on the receptor surface and that the ink is not offset so as to distort the image character.

Fusing devices which have been utilized for this image fixing generally include a pair of nip rolls, one being a heated fusing roller having a peripheral surface which has a low affinity for the fused or softened ink, and the other being a pressure or backup roll. The receptor element, generally a sheet of paper, bearing the particulate ink advances between the nip area of the rollers whereby the ink is to be fused and bonded to the receptor surface. The peripheral surface of the fusing roller must have a sufficiently low affinity for the softened ink such that the tacky ink particles preferentially adhere to the receptor surface rather than the fuser roll surface. If these particles do stick to the fuser roll surface, a splitting of the image occurs, such that a partial or ghost image results on the next advancing sheet, producing what is commonly termed in the duplicating art an offset image.

One approach to providing a surface for the fusing roller which has a low affinity for the softened ink is by using nip rolls which may be coated with a tetrafluoroethylene resin such as Teflon and a system for dispensing a silicone oil (a dimethyl siloxane polymer) onto the heated fusing roll, as taught by U.S. Pat. Nos. 3,291,466; 3,331,592; 3,449,548; and 3,452,181.

Another method, designed to eliminate problems encountered with liquid dispensing systems, is to provide a silicone elastomer surface for the heated fusing roll, as is taught in U.S. Pat. No. 3,669,707. However, the silicone elastomer surface is subject to abrasion and chemical interaction with the ink particles, which does cause a long-term loss in effectiveness.

A recent improved fusing device, as disclosed in copending and commonly assigned U.S. patent application, Ser. No. 103,725, filed by Gorka et al on Jan. 4, 1971, now U.S. Pat. No. 3,716,221 granted Feb. 13, 1973, utilizes a fusing blanket comprised of a thin, flexible heat-conductive substrate, such as stainless steel, having bonded thereto a silicone elastomer, which can be removably mounted on a heated fusing roll. During operation an offset preventing fluid, e.g. silicone oil, is applied to the silicone elastomer surface of the fusing blanket. The silicone elastomer surface is, however, somewhat penetrable by the offset preventing

liquid. It has been found that this penetration can tend to cause a failure of the bond between the heat-conductive substrate and the silicone elastomer overlayer over a period of time, eventually resulting in delamination of the blanket.

This invention provides a fusing blanket which retains the beneficial silicone elastomer surface for offset prevention and allows utilization of a dispensed fluid such as silicone oil without any attendant delamination problem. This is accomplished by providing a fuser blanket in the form of a composite construction of a heat-conductive substrate having bonded thereto, in ascending order, a fluorinated elastomeric polymer and a silicone elastomer. While the silicone elastomer is penetrable by offset preventing fluids such as silicone oil, the fluorinated elastomer is substantially impenetrable. Also, the bond between the silicone and fluorinated elastomers is not affected by penetration of the fluid. Thus delamination of the fuser blanket is effectively prevented, resulting in a longer-lived fuser blanket.

## SUMMARY OF THE INVENTION

In accordance with the invention, there is provided a composite article useful as a fuser blanket comprising a dimensionally stable heat conductive substrate having bonded to at least one surface thereof a thin, resiliently compressible layer of a fluorinated elastomeric polymer and a thin, resiliently compressible silicone elastomer outer layer bonded thereto.

The composite blanket can be conveniently utilized in high speed copier systems wherein an offset preventing fluid such as silicone oil is applied to the fusing roll because the fluid does not have a long term detrimental effect on the laminate structure, i.e. it does not promote delamination of the blanket during operation.

## DETAILED DESCRIPTION OF THE INVENTION

To illustrate the invention, accompanying drawings are presented wherein FIG. 1 is a simple schematic view of a fusing device wherein the fuser blanket is utilized, and FIG. 2 is a cross-section of the preferred fuser blanket.

Typically, the fuser device illustrated in FIG. 1 has a fusing roller 9, a backup roller 13, a toner offset preventing liquid applicator 16 and a backup roller cleaner 19.

The fusing roller 9 comprises a hollow drum 10 of a heat conductive material such as aluminum generally having a heat source therein (not illustrated) to provide sufficient heat to the periphery of the fusing blanket 11 covering the drum to fuse the ink 27 to the receptor sheet 26. The fused ink is shown as 28. The fusing blanket is preferably wrapped around the drum and attached thereto. The outer peripheral surface of the fusing blanket generally has about a 15 inch circumferential extent so as to permit fusing of developer to a 14 inch receptor sheet upon a single revolution of the fuser roll. The fuser roll has a shaft 12 connected thereto which can be utilized to drive the fuser roll.

Backup roller 13 comprises a hollow drum, typically of aluminum, with an exterior surface coating 14 of polytetrafluoroethylene providing a rigid peripheral surface. The backup roller has a shaft 15 connected thereto which can be used to drive the roller. Fusing pressure, i.e. the pressure required to force a receptor sheet 26 into intimate contact with fusing blanket 11, is

generally applied by the backup roller by convenient means such as, for example, compression springs.

The offset preventing fluid applicator comprises a receptacle 16 in which is contained an offset preventing liquid 17. A wick 18 extends from the fluid receptacle 16 toward backup roller 13 along the length thereof for applying the fluid.

The backup roll cleaner 25 comprises a supply roll 21 of a cleaning web 20, a takeup roller 19, and a drive for transferring the cleaning web 20 from supply roll 21 to takeup roller 19. Takeup roller 19 is biased into contact with backup roller 13 by any convenient method, e.g. springs. In use a fresh portion of cleaning web is continuously presented to backup roller 13 to remove excess offset preventing fluid 17 and any toner powder or other debris accumulated thereon.

In use, the fusing roller 9 is actuated as a receptor sheet containing imaged toner powder thereon approaches the nip area between fusing roller 9 and backup roller 13 and positions the receptor sheet. Fusing pressure is applied at the nip area by the backup roller 13 and heat is applied to the fusing blanket typically by a source within the fusing drum 10, thereby fusing the toner powder to the receptor sheet. Offset preventing fluid applied to the backup roller 13 can be transferred to the periphery of the fuser blanket 11 by permitting an occasional extra rotation of the fuser roller 9 and backup roller 13 without a receptor sheet therebetween.

FIG. 2 is a cross section of the preferred fuser blanket 11 of this invention, illustrating a backing member 24 of a dimensionally stable, heat conductive material having bonded thereto a thin fluorinated elastomeric layer 23 and bonded thereover a thin silicone elastomer overlayer 22 which is the surface of the blanket contacted by the offset preventing liquid and the fusible toner powder on a receptor sheet. Preferably the dimensionally stable heat conductive substrate is a thin, flexible metallic sheet material. However, the substrate can alternatively be the surface of fusing roller 10.

For commercial high speed duplicating systems a fuser blanket must typically possess certain characteristics. First, the blanket must be resiliently compressible so as to provide an area of intimate contact with the receptor when pressure is applied at the nip via the backup roller. Second, the blanket must be capable of withstanding pressures in excess of about 100 psi at operating temperatures in excess of about 200°C. while maintaining its physical and dimensional integrity over a long period of time. Third, the blanket surface must have a low affinity for the toner powder under fusing conditions. Fourth, the blanket must be capable of withstanding continuous contact with an offset preventing fluid such as silicone oil for a long period of time under the elevated temperatures encountered during fusing.

For high speed duplicating systems wherein extended blanket life is extremely desirable, silicone elastomers may not be capable of withstanding continuous contact with an offset preventing fluid such as silicone oil for the desired long period of time. Fluorinated elastomers, conversely, are capable of withstanding long term continuous contact with such fluids, as they are substantially impenetrable to such fluids. However, fluorinated elastomers generally do not have a sufficiently low affinity for toner powder under the conditions encountered during the fusing operation. By combining silicone and fluorinate elastomers, a composite is attained

wherein silicone oil or other offset preventing fluid will substantially penetrate only the silicone elastomer layer, thereby allowing the fuser blanket to retain its physical and dimensional integrity during operation under fusing conditions for a long period of time. The bond formed between the silicone and fluorinated elastomers is not deleteriously affected to any substantial extent by the fluid penetration, and the release surface thereby remains intact under copier operation conditions over the extended period of time required for high speed duplicating systems.

The backing material or substrate suitable for use in the fusing blanket must be dimensionally stable at elevated temperatures. Additionally, when fusing temperatures are attained by heating means within the fusing roller, the substrate must be heat conductive. While the surface of the fusing roller itself can be utilized as the substrate, it is preferred to utilize a separate substrate or backing material. This is because insertion of a replacement fusing blanket is simplified to a great extent. If the blanket is formed on the surface of the fusing roller, the entire roller must be replaced. Conversely, when a separate backing is utilized the blanket can be releasably attached to the fusing roller to facilitate replacement. Metallic sheet material is exemplary of suitable material possessing the aforementioned characteristics. A preferred backing is stainless steel, although materials such as aluminum, copper and brass are also satisfactory. Substrate thicknesses should be sufficient to provide strength and dimensional stability and yet be flexible enough to easily conform to the fusing roller. Generally, thicknesses in the range of about 2 mils to about 15 mils, preferably about 5 mils, are satisfactory. Decreasing thicknesses tend to provide greater flexibility, thereby facilitating conformance of the composite blanket to the fusing roller, but provide decreased strength and dimensional stability. Conversely, increasing thicknesses provide greater strength but less flexibility.

Fluorinated curable polymers useful in this invention are those which when cured to an elastomer are substantially impenetrable to offset preventing fluids such as silicone oil and which are resiliently compressible so as to provide intimate contact of the fuser blanket with a receptor surface. Additionally, the fluorinated elastomer should be heat transmissive when fusing temperatures are attained by heating means within the fusing roller. When heating means are utilized external from the fusing roller, this criteria is of course immaterial. Preferable fluorinated polymers are those containing at least about 37% by weight of carbon-bonded fluorine, and more preferably wherein at least about 50% of the non-skeletal carbon valance bonds are to fluorine. Exemplary of such polymers are fluorosilicone polymers which can be generally termed perfluoro alkyl alkylene siloxanes. These polymers contain a terminal perfluoro alkyl group which is positioned no closer than two carbon atoms from the silicon atom, and additionally contain a minor amount of substituent groups which will allow curing or crosslinking to occur. These substituent groups can for example be silicon-bonded hydrogen atoms, vinyl groups, or peroxy-activatable groups. A preferred curable fluorosilicone polymer is commercially available from the Dow Corning Co. under the tradename LS-53, which is a trifluoropropyl methyl vinyl polysiloxane.

Linear saturated fluorinated copolymers of vinylidene fluoride and fluoromonolefins, as disclosed in

U.S. Pat. No. 3,655,727 are also exemplary of suitable curable fluorinated polymers. Preferred saturated fluorinated polymers are those produced by copolymerizing perfluoropropene and vinylidene fluoride as described in U.S. Pat. Nos. 3,051,677 and 3,318,854.

The fluorinated elastomer layer should generally have a thickness sufficient to provide a resiliently compressible and, if required, heat transmissive layer, typically from about 10 mils to about 100 mils, and preferably about 30 mils.

The softness of this elastomer layer should be sufficient to provide suitable nip contact area during the fusing operation and yet maintain physical integrity. Generally, an elastomer having a Shore A durometer hardness of 20 to 80, and preferably 50 is satisfactory.

The fluorinated elastomer layer can be conveniently formed by curing the fluorinated polymers in situ at the time of manufacture of the blanket. Curing or cross linking agents for curing fluorinated polymers are generally well known in the art. For example, curing systems for vinylidene fluoride/ fluoromonoolefin elastomeric copolymers are taught in U.S. Pat. No. 3,655,727. Curing or cross linking agents for use with curable fluorosilicone polymers include dicumyl peroxide, 2,4-dichlorobenzoyl peroxide, benzoyl peroxide, di-tertiarybutyl peroxide, tertiary-butyl perbenzoate, and 2,5-dimethyl2,5 di(t-butyl peroxy) hexane. Curing conditions vary depending upon the curable fluorinated polymer and curing agent chosen, effective cures being obtained at temperatures up to about 450°F. for a period of from about 1 minute to about 15 hours, and more usually from about 5 minutes to about 30 minutes.

Silicone elastomers suitable for use in this invention are characterized and described in U.S. Pat. No. 3,554,836, granted to Steindorf on Jan. 12, 1971, incorporated herein by reference the adhesive nature of such elastomers are quantitatively characterized therein by their release values. As indicated therein, silicone elastomers customarily have release values of less than about 30 grams/inch. Furthermore, materials having release values greater than 100 grams/inch will not release thermoplastic transfer media to a receptor in nonsplitting fashion. Exemplary silicone elastomers include the cured or further polymerized product of a silicone gum, such as dimethyl vinyl polysiloxane sold under the tradename SE-33. The preferred blanket surface comprises an elastomer prepared from a mixture of the above-mentioned gum with a silicone resin such as sold under the tradename Sylgard 184, with equal parts by weight of the gum and resin being the preferred mixture. However, other proportions of these ingredients are also useful. For example, from 30 to 100 parts by weight of gum with correspondingly from 70 to 0 parts by weight of resin will produce a useful blanket surface. A cured surface composed of the silicone resin containing less than 30 percent by weight of the silicone gum may be too hard to be useful in this invention.

For the preparation of the silicone elastomer layer, curing agents such as benzoylperoxide, 2,4-dichlorobenzoyl peroxide, tertiarybutyl perbenzoate, dicumyl peroxide or the like are satisfactory. Preferably the curing agent is a mixture of low molecular weight polydimethyl siloxane containing silane groups and an initiative catalyst, such as the curing agent being sold under the tradename "Sylgard 184 Curing Agent." Curing conditions required by these agents vary de-

pending upon the curing agent and the silicone gums or resins, effective cures being obtained at temperatures up to 400°F.

The silicone elastomer thickness should be sufficient to permit adequate wear life in terms of abrasion resistance without excessive swelling due to contact with an offset preventing fluid such as silicone oil. Typically, about 0.3 mils to about 10 mils is satisfactory, with 4 mils being preferred.

10 The hardness of the silicone elastomer should be such as to allow sufficient elongation without tensile failure, typically in the range of about 10 to about 70 Shore A durometer, preferably 30 Shore A durometer. An elastomer prepared from equal parts of the aforementioned silicone gum and resin typically has a Shore A durometer value of 20-30, a tensile strength of 370 psi, percent elongation at break of 24, and a tear strength of 60 psi.

15 In the manufacture of the fuser blanket of this invention, the stainless steel or other suitable backing member generally must be primed with a suitable primer for fluorinated elastomers to insure an adequate bond surface for the fluorinated elastomer and to insure reliable repeatability of attained bond strength. The result desired is cohesive failure of the fluorinated elastomer layer before adhesive failure of the fluorinated elastomer-backing member interface when subjected to a conventional bond test such as a 90° or 180° peel test. Such primers are commercially available. A preferred primer

20 when fluorosilicone elastomers are utilized is that commercially available under the tradename Dow Corning A-4040 from the Dow Corning Corporation. The primer can be applied to the substrate in a conventional manner, and can be conveniently applied from a solution of a suitable volatile solvent, such as V.M.&P. Naphtha. Recommended conditions for application are generally indicated by the manufacturer. For example, when utilizing the Dow Corning A-4040 mentioned above, the recommended application environment is 70°F. and 50 percent relative humidity. A one hour air dry under these conditions, or a 5 minute air dry followed by 5 minutes at 300°F. will effectively cure the applied primer.

25 40 45 With the curable fluorinated vinylidene fluoride/ fluoromonoolefin copolymers, an acceptable bond can be obtained utilizing as a primer an adhesive sold under the tradename Chemlok No. 607 by the Hugheson Chemical Co. Similarly, a primer consisting of equal parts of a 50 weight percent solution of Chemlok No. 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 977

convenient manner, such as spraying, knife coating, brush coating, or dip coating. A preferred application method is by spraying a solution of the curable catalyzed silicone composition in a volatile solvent such as heptane, toluene, or xylene. The concentration of the silicone composition in an application solution can generally be from about 10 to about 20 weight percent when spraying is utilized, or about 50 weight percent or greater when coating is the application method utilized.

It may be advantageous to prime the cured fluorinated elastomer layer prior to application of the curable silicone composition thereto. In such cases the aforementioned Dow Corning A-4040 fluorosilicone rubber primer has been found to be an excellent primer.

The curable silicone composition overlayer and the composite blanket can then be cured and postcured at about 400°F. for from about 4 hours to about 24 hours. Postcuring of the composite structure is desired to develop high temperature stability and to maximize the physical properties of the blanket.

The toner powders to be fused to the receptor sheet utilizing the fuser blanket of this invention are generally heat fusible materials in particulate form with an average particle size of about 7 microns. A typical suitable toner powder has the following composition in percentages by weight:

|     |                                                                                    |
|-----|------------------------------------------------------------------------------------|
| 44% | Epon 1004 (tradename for an epoxy resin available from the Shell Chemical Company) |
| 52% | magnetite                                                                          |
| 4%  | carbon black                                                                       |

Another suitable developer powder consists of 65 weight percent polystyrene and 35 weight percent carbon black.

The temperature at which the fusing blanket operates may vary from about 50°C. to about 200°C. depending upon the choice of toner powder and the desired rate of fuser operation.

In order to more clearly illustrate the invention, the following nonlimiting examples are provided wherein all parts are by weight unless otherwise specified.

#### EXAMPLE 1

A primer solution is prepared as follows:

|          |                                                                                                        |
|----------|--------------------------------------------------------------------------------------------------------|
| 50 parts | Dow Corning A-4040 (tradename for a fluorosilicone rubber primer available from the Dow Corning Corp.) |
| 50 parts | V.M.&P. naphtha                                                                                        |

One surface of a 5 mil thick stainless steel sheet (Type 302 stainless with a number 2 finish,  $\frac{1}{4}$  hard) is primed with the primer solution by brushing at about 75°F. and at a relative humidity of about 50 percent. The primer is allowed to dry for one hour at these same conditions.

A catalyzed fluorosilicone polymer is prepared by mixing on a conventional rubber mill

|            |                                                                                        |
|------------|----------------------------------------------------------------------------------------|
| 0.72 parts | Dicup R (tradename for dicumyl peroxide, available from the Hercules Chemical Company) |
| 100 parts  | LS53 Fluorosilicone Rubber (tradename for a Dow Corning Corp. fluorosilicone)          |

The catalyzed polymer is applied to the primed side of the stainless steel sheet in a preform fashion and inserted into a 290°F. conventional compression mold. The fluorosilicone polymer is cured at 350 psi for 7 minutes in the mold. The thickness of the cured fluorosilicone elastomer layer is 30 mils.

A spray solution of catalyzed silicone gum and resin is prepared by dissolving

|    |          |                                                                                                                      |
|----|----------|----------------------------------------------------------------------------------------------------------------------|
| 10 | 2 parts  | Dow Corning No. 184 Sylgard (tradename for a silicone encapsulating resin available from the Dow Corning Corp.)      |
| 15 | 2 parts  | General Electric SE 33 (tradename for dimethyl vinyl silicone gum available from the General Electric Company)       |
| 20 | 1 part   | Dow Corning No. 184 Catalyst (tradename for silicone encapsulating resin curing catalyst from the Dow Corning Corp.) |
| 20 | 45 parts | heptane                                                                                                              |

The solution is applied to the cured fluorosilicone elastomer by conventional spraying in a spray booth.

The silicone composition is cured and the composite fuser blanket is postcured simultaneously for 4 hours in a 400°F. environment. The thickness of the cured silicone elastomer layer is 4 mils.

The composite fusing blanket is mounted on a fuser device as illustrated in FIG. 1 whereupon 150,000 copies (8- $\frac{1}{2}$  in.  $\times$  14 in.) are fixed over a 90 day period prior to the need for replacement of the composite blanket. The fuser blanket is contacted with silicone oil during the operation of the copier. The temperature of the silicone elastomer surface of the fuser blanket is typically 375°F. and the softening point of the toner is 160°F.

#### EXAMPLE 2

One surface of a 5 mil thick stainless steel sheet (Type 302 stainless with a number 2 finish,  $\frac{1}{4}$  hard) is primed with Chemlok No. 607 (tradename for primer system, available from the Hugheson Chemical Co.) by brushing at about 75°F. and at a relative humidity of about 50 percent. The primer is allowed to dry for 30 minutes at these same conditions.

A curable fluorinated polymer composition is prepared by mixing

|    |           |                                                                                                                                          |
|----|-----------|------------------------------------------------------------------------------------------------------------------------------------------|
| 50 | 30 parts  | Thermax MT (tradename for carbon black available from the R. T. Vanderbilt Co.)                                                          |
|    | 3 parts   | Maglite D (tradename for magnesium oxide available from the Merck Company)                                                               |
|    | 6 parts   | Calcium hydroxide                                                                                                                        |
|    | 100 parts | Fluorel 2170 (tradename for a vinylidene fluoride/propylene copolymer and available from the Minnesota Mining and Manufacturing Company) |

The catalyzed polymer composition is applied to the primed side of the stainless steel sheet in a preform fashion and inserted into a 350°F. conventional compression mold. The polymer is cured at 350 psi for 5 minutes minimum in the mold. The thickness of the cured fluoroelastomer layer is 30 mils.

The cured fluoroelastomer layer is primed by brushing with a primer solution of 50 weight percent Dow Corning A-4040 in V.M.&P. naphtha at about 75°F.

and a relative humidity of about 50 percent, followed by drying for one hour at these same conditions.

After cutting the fluorinated elastomer coated stainless steel sheet to the desired size, the same curable silicone composition as in Example 1 is applied to the primed fluorinated elastomer surface in the same manner as in Example 1. The silicone composition is then cured and the composite blanket is postcured simultaneously for 24 hours in a 400°F. environment.

When utilized in an electrophotographic office copier wherein silicone oil is contacted by the fuser blanket, results similar to Example 1 are achieved.

An accelerated testing program was utilized to compare the fusing blanket of this invention with a blanket construction having a silicone elastomer bonded to a stainless sheet. This program utilized a test fusing device comprising a separate fusing module substantially as shown in FIG. 1 of the accompanying drawing. The fusing roll and the backup roll were continuously rotated while maintaining nip pressure and the fuser blanket was continuously heated from within the fusing roll. No receptor sheet was utilized and a silicone oil film was continuously maintained on the fusing blanket periphery. The blanket surface temperature was maintained at approximately 375°F.

One surface of a 5 mil thick stainless steel sheet (Type 302 with a number 2 finish, 1/4 hard) is primed by brushing with Dow Corning S-2260 primer at 75°F. and 50 percent relative humidity, followed by a one hour air dry under these conditions.

A catalyzed curable silicone composition is prepared by mixing:

|           |                                                                                               |
|-----------|-----------------------------------------------------------------------------------------------|
| 0.4 parts | dicumyl peroxide                                                                              |
| 100 parts | GE No.24514 (a curable methyl phenyl silicone rubber available from the General Electric Co.) |

The catalyzed silicone composition is applied to the primed side of the stainless steel sheet in a preform fashion and cured in a 300°F. conventional compression mold for 8 minutes. The thickness of the cured silicone elastomer layer is 30 mils. The blanket is postcured for 4 hours at 400°F.

This blanket construction, when utilized in the accelerated testing program, has an average lifespan of 20 hours prior to delamination of the silicone elastomer from the backing.

Conversely, the lifespan of a fusing blanket prepared as per the illustrative examples averaged in excess of 348 hours under the same accelerated conditions.

What is claimed is:

1. A composite article suitable for use as a fuser blanket comprising a dimensionally-stable substrate having bonded to one surface thereof a thin, resiliently compressible layer comprising a fluorinated elastomer, and overlying said fluorinated elastomer and bonded thereto a thin, resiliently compressible layer comprising a silicone elastomer, said silicone elastomer having a release value of less than 100 grams per inch.

2. The article of claim 1 wherein said fluorinated elastomer is a fluorosilicone elastomer.

3. The article of claim 1 wherein said fluorinated elastomer is a cured linear saturated copolymer of vinylidene fluoride and at least one fluoromonoolefin.

4. The article of claim 3 wherein said fluoromonoolefin is perfluoropropene.

5. The article of claim 1 wherein said fluorinated elastomer contains at least about 37 weight percent of carbonbonded fluorine.

6. The article of claim 1 wherein said dimensionally stable substrate is comprised of a thin, flexible, metallic sheet material.

7. The article of claim 6 wherein said sheet material is stainless steel.

\* \* \* \* \*